

Patented June 13, 1939

2,162,207

## UNITED STATES PATENT OFFICE

2,162,207

## LUBRICATING OIL

Robert C. Moran, Wenonah, and William H. James, Paulsboro, N. J., assignors to Socony-Vacuum Oil Company, Incorporated, New York, N. Y., a corporation of New York

No Drawing. Application June 5, 1937,  
Serial No. 146,595

## 1 Claim. (Cl. 87-9)

This invention is directed broadly to the provision of oils for use in automotive engines of modern design, using the newer hard metal bearings, which are in general more susceptible to corrosive agencies under conditions of use.

Recent changes in automotive engine design, tending toward higher bearing pressures, higher rotative speeds, higher engine temperatures, and the like, have occasioned departure from the use of the usual bearing metals such as babbitt. The newer bearing metals are of different nature and, while harder, are in general more susceptible to destructive agencies of a corrosive nature. Typical of these newer bearings are those composed of a cadmium-silver alloy supported upon a steel back, which are now widely installed in certain makes of automobiles. Others of these relatively new bearing metals which may be mentioned are cadmium-nickel and copper-lead alloys, and so-called high lead bearings.

These changes in engine design have been concurrent with marked advances in methods of refining lubricant oils for automotive use. The demand for oils having lesser changes in viscosity with temperature change; i. e., higher viscosity index (V. I.) has been met by refining lubricants intended for motor oils by certain solvent refining or solvent extraction processes, wherein advantage is taken of the selective solvent power for hydrocarbons of various types which is possessed by certain liquid reagents, for example, dichloro-diethylether, cresylic acid, phenol, chloraniline, chlorophenol, phenetidine, benzyl alcohol, nitro-benzene, benzonitrile, furfural, aniline, benzyl acetate, liquid sulphur dioxide, mixtures of liquid sulphur dioxide or aniline with benzol, and the like. These solvent refining processes are operated to concentrate in the desired lubricant fraction those compounds of a "paraffinic" nature possessed of the ability to suffer only a small change in viscosity upon change of temperature, and to reject the compounds of "naphthenic" nature which do suffer such change of viscosity to a more marked degree. These refining processes have enabled supply of an oil of quite desirable general characteristics, definitely far superior to any oil previously produced from mixed base or asphaltic crudes, and superior to a like, though lesser, degree over oils previously produced from paraffin base crudes.

It has been found that the solvent refined motor oils referred to above are for some reason definitely corrosive to the newer bearing metals under normal conditions of automotive use, sometimes resulting in bearing failure after only a few thousand miles of normal driving. It is further known that the same reaction, viz., corrosion of alloy bearing metals such as cadmium-silver, also occurs in good paraffinic base oils which have not been subjected to solvent refining. The higher the V. I. of the lubricating oil, the more pronounced is the tendency to corrosion of the kind referred to above. Generally speaking, the problem is encountered in oils having a V. I. of 75 or higher, and becomes important in oils having a V. I. of 80 to 85 or higher, and very important in oils of 100 V. I. or higher.

It is an important object of this invention to provide means for satisfactorily inhibiting or preventing this corrosion from taking place to a serious degree. It is an object of this invention to alter or modify a highly refined motor oil, normally corrosive, by the use of an additive ingredient capable of substantially inhibiting this corrosion. It is an object to provide a substantially non-corrosive motor oil of high V. I. An object of this invention is to provide an additive reagent or ingredient capable of inhibiting the corrosive properties of these oils. The production of solvent refined oils of low corrosive properties under conditions of automotive use is a major object of this invention, as well as the method of production of such oils which couple high viscosity index with low tendency to corrosion.

This invention is based on the discovery that the above objects may be accomplished by the addition to the motor oil of small amounts of aryl amino polysulphides. It is found that when corrosion of the type outlined above on the bearings of the type outlined above occurs, that the corrosion can be inhibited and that the oil can be rendered substantially non-corrosive under conditions far more strenuous than normal driving conditions, by the addition of controlled amounts of these compounds, and particularly by the addition of controlled amounts of aniline disulphide.

The reaction products of aryl amines and elementary sulphur are those compounds to which this invention is directed, the preferred member

## Cross Reference

391 2

2,162,207

of this group being aniline disulphide. These compounds have the following general formula  $(\text{NH}_2\text{C}_6\text{H}_4)_2\text{S}_x$  where R is a hydrogen atom and/or an alkyl group and S<sub>x</sub> may represent 1, 2, 3, or 4 sulphur atoms. The grouping  $(\text{NH}_2\text{C}_6\text{H}_4)$  corresponds to aniline or to an alkyl-substituted aniline residue. These compounds are generally prepared by the interaction of an aniline compound and elementary sulphur. Thus dianiline disulphide can be prepared from the interaction of aniline and sulphur after the following scheme:



In other words when 2 moles of aniline and 3 atoms of sulphur are mixed and heated until the temperature of the reaction mixture is about 190° to 195° C., a reaction occurs with the evolution of 20 hydrogen sulphide. The first disulphide product of the reaction is 2,2' diamino diphenyl disulphide, but 4,4' diamino diphenyl disulphide is formed in increasing proportions as the temperature rises. There is also some formation of the 25 3,3' diamino diphenyl disulphide. The unreacted aniline may be removed from the reaction mixture by steam distillation. The unreacted sulphur may be removed from the reaction mixture by converting the aniline sulphide products to their 30 hydrochlorides and extraction with hot water. The hydrochloride salt extract then yields the free aniline sulphur complex when neutralized with a base such as sodium hydroxide. The methods of synthesis and purification to form 35 these products are well known in the art of chemical synthesis. The aniline sulphur complex thus obtained consists mainly of a mixture of isomeric aniline disulphides. The crude product as obtained melts at 72-84° C. According to the 40 literature, the isomeric 2,2' diamino diphenyl disulphide melts at 93° C., the 3,3' isomer melts at 59-60° C., and the 4,4' isomer melts at 81 to 82° C. From the above evidence, it is apparent to those skilled in the art that the product above 45 obtained consists mainly of a mixture of the various isomeric forms of diamino diphenyl disulphide, although it is possible that some compounds of other nature are present therein in small amounts. The crude product of the above-50 outlined synthesis melting at 72 to 84° C. has been found to be effective ingredient to prevent the corrosive action of motor oils on hard metal bearings when subjected to strenuous use at high temperatures for prolonged times. This material 55 is hereinafter referred to as aniline disulphide.

It is also possible to prepare other compounds having similar effectiveness when one or more nuclear hydrogens of the aniline member are substituted with alkyls such as methyl or ethyl 60 radicals.

The following sets of data demonstrate the effectiveness of this novel corrosion inhibitor. In all of these tests, the oil used was a solvent refined motor oil of S. A. E. 20 rating, having a 65 Saybolt viscosity of 55.3 seconds at 210° F., a flash point of 435° F. Actual motor operation tests are set forth in Table I, below. In these tests, a motor oil blank and motor oil blends containing different proportions of the novel inhibiting ingredient of this invention were subjected to test in a modified Delco knock test engine, equipped with bearings of cadmium-silver alloy on a steel back. The alloy is about 2.5% silver, 70 a few hundredths of a per cent of copper, and the 75

balance of cadmium. The motor was equipped with crankcase oil heaters to maintain oil-temperatures (330° F.) at least equal to those encountered under extreme conditions of automotive use. On each test the test engine was operated for at least 20 hours at a rotative speed the equivalent of an automobile road speed of 60 miles per hour. In rough terms, each 20 hours of test is the equivalent of exposure of the oil to use in an automobile for 1200 miles of continuous 60-mile-an-hour driving, a condition far more rigorous than any encountered in normal use. The bearings in the engine were new for each test, and were carefully weighed before and after to determine loss in weight. The neutralization-number (N. N.) of the used oil was measured, and is recorded as being indicative of the corrosive nature of the oil.

| Time (hours) of engine operation | Bearing loss, mg. |                                | Neutralization No. |                                |
|----------------------------------|-------------------|--------------------------------|--------------------|--------------------------------|
|                                  | Oil alone         | Oil + 0.25% aniline disulphide | Oil alone          | Oil + 0.25% aniline disulphide |
| 20 hours.....                    | 1,328             | 107                            | 3.0                | 1.2                            |
| 40 hours.....                    |                   | 145                            | .....              | 2.3                            |
| 60 hours.....                    |                   | 879                            | .....              | 5.7                            |

  

|               | Oil alone | Oil + 0.10% aniline disulphide | Oil alone | Oil + 0.10% aniline disulphide |
|---------------|-----------|--------------------------------|-----------|--------------------------------|
| 20 hours..... | 1,328     | 95                             | 3.0       | 1.0                            |
| 40 hours..... |           | 798                            | .....     | 3.1                            |

From this it may be seen that the use of this novel corrosion inhibitor, viz., aniline disulphide, in amounts as small as  $\frac{1}{4}$  of 1% prevented corrosion to a substantially complete degree under conditions far more rigorous than any to be met in practice, while as little as  $\frac{1}{10}$  of 1% reduced the bearing loss almost one-half.

An indicative test of considerable merit may be made in the laboratory by suspending a portion of a cadmium-silver alloy bearing in a bath of the oil under test in a glass container, maintaining the oil at about 350° F., and passing air through the oil in contact with the bearing metal. Convenient conditions are as follows: 30 gm. oil, 2,000 ml. air per hour, 22 hours. The following table shows results of a series of such tests in which oils containing different proportions of aniline disulphide, and an oil blank were tested, giving the loss in weight of the bearing metal. The oil used was the same as in Table I:

Table II

| Percent of aniline disulphide in oil | Loss in weight of bearing, mg. |                                              |
|--------------------------------------|--------------------------------|----------------------------------------------|
|                                      | Oil alone                      | With indicated percent of aniline disulphide |
| 0.25.....                            | 38                             | 0                                            |
| 0.10.....                            | 96                             | 0                                            |
| 0.05.....                            | 62                             | 1                                            |
| 0.01.....                            | 62                             | 60                                           |

From the combined evidence of the exemplary data set forth above, it is evident that the novel inhibiting ingredients herein disclosed, viz., aniline disulphide and alkyl-substituted aniline disulphides are effective agents for the prevention of corrosion under conditions of use of automotive parts, particularly of the newer type alloy

bearings, when introduced in proper amounts into an oil otherwise highly corrosive.

It is preferred to use these ingredients in amounts ranging between 0.25% to 1.0% by weight, although for less severe service and in oil not highly corrosive in nature, as low as 0.10% may be fully effective for the purposes intended.

That the oils protected by the novel inhibiting agent herein disclosed, viz., aniline disulphide, are also effective to protect copper lead bearings, may be shown by the following tests wherein an engine test under conditions similar to those outlined in the Delco engine test described above was conducted in a Cooperative Fuel Research engine (commonly known in petroleum and automotive laboratories as a C. F. R. engine), equipped for the purposes of test with copper lead bearings of the type commonly used in automotive engines of new designs. In these tests, the oil used was an oil of the following specifications:

Gravity..... °A. P. I. 27.5  
 Flash..... °F. 500  
 Viscosity..... Saybolt at 210° F. 115 to 120''  
 Viscosity-index..... 100

In the following tabulation a comparison is shown between this oil, used alone for 40 hours, and the same oil to which had been added 0.125% by weight of aniline disulphide, and exposed to conditions of engine operation for 60 hours.

Table III

| Time (hours) engine operation | Bearing loss, mg. |                               | Neutralization No. |                               |
|-------------------------------|-------------------|-------------------------------|--------------------|-------------------------------|
|                               | Oil alone         | Oil+0.125% aniline disulphide | Oil alone          | Oil+0.125% aniline disulphide |
| 40.....                       | 1.223             |                               | 11.4               |                               |
| 60.....                       |                   | 1.699                         |                    | 12.0                          |

From the above tabular data it may be noticed that the additive agent is quite effective in this case, enabling the oil to achieve results at the end of 60 hours' operation when protected, that were comparable with the results obtained at the end of 40 hours' operation with an unprotected oil.

We claim:

A method of lubricating bearing surfaces which comprises maintaining between the bearing surfaces, one of which contains a characterizing proportion of cadmium, silver, nickel, copper, or lead, a film of lubricating oil which initially produces an effective lubricating action, but would normally tend to corrode the adjacent surface, and maintaining the effectiveness of the lubricating oil by incorporating therein dianiline disulphide in a small but sufficient proportion to substantially retard the corrosion.

ROBERT C. MORAN. 30  
 WILLIAM H. JAMES. 25